

# United States Patent Office

2,852,465

Patented Sept. 16, 1958

1

2,852,465

## STEAM TURBINE LUBRICANT

Hans C. H. Jensen, East Hendred, near Wantage, England, assignor to Esso Research and Engineering Company, a corporation of Delaware

No Drawing. Application November 26, 1954  
Serial No. 471,529

Claims priority, application Great Britain  
December 9, 1953

2 Claims. (Cl. 252—33.4)

This invention relates to new and improved lubricants particularly adapted for the lubrication of steam turbines. The lubricants of this invention are characterised by their freedom from forming stable emulsions on agitation with water.

The steam turbine is an increasingly popular prime mover and is particularly useful for marine propulsion. The lubrication of the steam turbine however presents a number of problems. The turbine itself has a very high speed and therefore there must be associated with it a reduction gear-box to reduce the number of revolutions per minute transmitted to the propeller.

The lubricant in a steam turbine circulates through the system and during circulation inevitably comes in contact with water. In the system it is normal to have a separator to separate any entrained water, and it is essential that the lubricant frees itself of all entrained water in this separator. The separator is usually either a filter, a centrifuge or a separating drum.

Generally speaking, since the lubricant has to be circulating in the system for a considerable length of time

2

reduce this tendency to form emulsions. Thus this invention comprises a lubricating oil composition adapted to lubricate steam turbines containing a small proportion of a sulphonated fatty acid.

- 5 The amount of sulphonated fatty acid that should be added is quite critical, but is readily determined by experiment. It is normally less than 5% and preferably is in the range of 0.001 to 0.2%; the proportions in excess of 2% should be observed with care since in these cases 10 the sulphonated fatty oil may in fact promote emulsion formation.

To determine the proportion of sulphonated fatty oil to be used, all that is required is that the oil and the sulphonated material should be agitated with water and 15 the separation of the resulting emulsions should be noted.

- Generally speaking any fatty oil may be sulphonated to produce a useful additive according to the present invention. However, castor oil is the preferred fatty oil and the product of sulphonation Turkey-red oil, is very 20 well-known commercially. This may be and commonly is partially or completely neutralised to make a proportion of the alkali metal salt, e. g. sodium or potassium, or the ammonium salt.

- 25 The efficacy of this invention is manifest from the accompanying table, wherein the effect of 1% of Turkey-red oil is given on 4 turbine oil compositions:

### Results of laboratory demulsibility tests

- 30 *Test procedure.*—20 ml. of tap water and 180 ml. test oil are emulsified in a Sunbeam Mixmaster for 10 minutes at max. R. P. M. The emulsion formed is centrifuged in a Gallenkamp centrifuge for 10 minutes at max. speed (g-value=1,000). All operations are carried out at room 35 temperature.

| Code | Test Oil                       |                                      | Additives                                                                                                                                                                                              | Test Result;<br>Amount of<br>Sludge |
|------|--------------------------------|--------------------------------------|--------------------------------------------------------------------------------------------------------------------------------------------------------------------------------------------------------|-------------------------------------|
|      | Type                           | Base Oil                             |                                                                                                                                                                                                        |                                     |
| A    | OM-88.                         | Unknown.                             | Unknown.                                                                                                                                                                                               | Considerable.                       |
| B    | A + 0.1% T. R. O. <sup>1</sup> | do.                                  | do.                                                                                                                                                                                                    | None.                               |
| C    | OM-100.                        | do.                                  | do.                                                                                                                                                                                                    | Considerable.                       |
| D    | C + 0.1% T. R. O.              | do.                                  | do.                                                                                                                                                                                                    | None.                               |
| E    | E. P. Turbine Oil.             | Solvent extracted<br>distillate oil. | 0.4% 2,4-di t butyl p cresol. 0.1% polyethylene glycol<br>400 di-tri-ricinoleate. 0.05% Proprietary rust prevent-<br>ive. 0.001% silicone antifoam agent. 2% Tributyl<br>phosphate. 1.2% isopropylate. | Considerable.                       |
| F    | E + 0.1% T. R. O.              | do.                                  | do.                                                                                                                                                                                                    | None.                               |
| G    | E. P. Turbine Oil.             | do.                                  | 0.4% 2,4-di t butyl p cresol. 0.05% polyethylene glycol<br>di-tri-ricinoleate. 1% hexachlorocyclo hexane.                                                                                              | Considerable.                       |
| H    | G + 0.1% T. R. O.              | do.                                  | do.                                                                                                                                                                                                    | None.                               |

<sup>1</sup> Turkey-red oil.

it is necessary for it to contain various additives. These additives are required in order to reduce the oxidation tendencies of the oil under the high temperature oxydation conditions to impart to the lubricating oil properties that will result in the metal surfaces with which it is in contact being resistant to corrosion, to reduce its tendency to foam and to increase its ability to lubricate highly loaded gears and bearings.

A disadvantage of these additives is that generally speaking, whereas they fulfil their prime function satisfactorily, they tend to incite the lubricant to form emulsions in the presence of water. These emulsions are sometimes very intractable and result in the separating system functioning imperfectly. As a result water can circulate in the system and considerable damage can be done, and in some cases the separator clogs and the system suffers from oil starvation.

It has now been discovered and it is the subject of this invention that certain sulphonated fatty acids when added in controlled proportions to such turbine oils considerably

55 It will be seen that whereas with each of the 4 typical turbine oils tested a considerable sludgy emulsion of doughy consistency was formed on the interface between the oil and water layers, with the use of Turkey-red oil this emulsion was eradicated.

The base oil with which this invention is concerned can be any conventionally used mineral oil adapted for 60 the lubrication of steam turbines. That is to say it should contain additives to impart resistance to oxidation and it should contain additives to protect from corrosion metal surfaces with which it comes in contact.

The anti-oxidant will normally be a phenol or sub-65 stituted phenol or amine or organic sulphur containing compound. It is particularly preferred to use alkylated cresols for example 2,4-di t butyl p cresol. The rust preventative additives are organic polar compounds soluble in mineral oil. They normally comprise a molecule 70 having a hydrophobic and a hydrophilic portion.

What I claim is:

1. In a mineral oil composition, adapted for lubrica-

tion of steam turbines, comprising a blend of a solvent extracted distillate oil, an oxidation inhibiting amount of 2,4 di t butyl p cresol, a foam inhibiting amount of hexachlorocyclo hexane, and a rust inhibiting amount of polyethylene glycol di-tri-ricinoleate, wherein the presence of said inhibitors tend to incite emulsion formation, the improvement which comprises the addition to said lubricating compound a minor proportion, sufficient to reduce the emulsifying tendency of said composition, of a sulfonated castor oil.

2. The improvement according to claim 1, wherein said oxidation inhibiting amount constitutes 0.4% 2,4, di t butyl p cresol, said foam inhibiting amount constitutes 0.05% polyethylene glycol di-tri-ricinoleate and said rust inhibiting amount constitutes 1% hexachlorocyclo hexane.

## References Cited in the file of this patent

## UNITED STATES PATENTS

|   |           |                |       |               |
|---|-----------|----------------|-------|---------------|
| 5 | 1,677,389 | Howes          | ----- | July 17, 1928 |
|   | 2,390,491 | Bennett        | ----- | Dec. 11, 1945 |
|   | 2,390,492 | Bennett        | ----- | Dec. 11, 1945 |
|   | 2,528,466 | Borsoff et al. | ----- | Oct. 31, 1950 |

## OTHER REFERENCES

- 10 "Performance of Lubricating Oils," by Zuidema, Reinhold Pub. Co., 1952, pages 129-135 pertinent.  
 "National Advisory Committee for Aeronautics Wartime Report," Foaming of Aircraft-Engine Oils, September 1944, as Advance Restricted Report 4, 105, pages 65 and 74 pertinent.